

# UNITED STATES PATENT OFFICE.

JOSEPH GRENVILLE MELLEN AND WILLIAM FRANCIS MELLEN, OF BRIDGEPORT,  
CONNECTICUT.

## PROCESS OF MAKING ALUMINUM AND COPPER ALLOYS.

982,218.

Specification of Letters Patent. Patented Jan. 17, 1911.

No Drawing.

Application filed February 14, 1910. Serial No. 543,778.

*To all whom it may concern:*

Be it known that we, JOSEPH GRENVILLE MELLEN and WILLIAM F. MELLEN, citizens of the United States, residing at Bridgeport, county of Fairfield, State of Connecticut, have invented an Improvement in Processes of Making Aluminum and Copper Alloys, of which the following is a specification.

This invention relates to a new and useful process of compounding aluminum with other metals either precious or basic, and has for its object to produce a composite metal or alloy consisting primarily of aluminum and copper, iron, silver, nickel or any of the other metals, one or more of them, which shall possess the qualities of malleability and ductility to a degree that it has been heretofore impossible to produce in composite metals containing aluminum.

It is of course well understood by those familiar with the metallurgical art that while it would be extremely desirable to utilize the color and lightness of aluminum in composite metals or alloys requiring malleability and ductility it has been found practically impossible to procure a composite metal containing an appreciable quantity of aluminum and having these qualities to the desired extent. We have found that this lack of malleability and ductility in composite metals containing aluminum is due to the lack of thoroughness in compounding the two or more metals and the consequent lack of homogeneity in the resulting alloy. Our novel process overcomes this difficulty and produces a composite metal having its specific gravity lessened to a greater or less extent and its color modified by the presence of aluminum and also having the qualities of malleability and ductility to any required extent within reasonable limits.

With these and other objects in view we have made numerous experiments in the compounding of aluminum with various other metals which we term for convenience the foundation metal, greatly varying the proportions of aluminum depending upon the metal or metals with which it was compounded and the relative degree of malleability or ductility required for various uses. It may be stated as a general proposition that the greater the proportion of aluminum used the lighter will be the composite metal both in color and weight, and also the harder

and less malleable and ductile. By decreasing the proportion of aluminum the composite metal will be rendered heavier and usually darker in color but more malleable and ductile.

In carrying out our novel process the foundation metal weighed to the proportions desired is placed in a pot and melted. After the temperature of the metal has been raised above the melting point, a suitable quantity of aluminum is added thereto. As soon as the aluminum is melted a suitable oxidizing agent, for example, potassium bichromate preferably powdered, and a suitable flux, for example, borax, are added in the proportions approximately of one-half pound of potassium bichromate and one-quarter pound of borax to one hundred pounds of metal. The mixed chemicals are now seen to melt and boil furiously, then gradually the boiling ceases and a crust forms upon the surface of the molten mass. This crust immediately upon forming is broken with a stirrer and the whole mass is stirred. The remnants of the chemicals are volatilized and pass off through the flue, but should a small amount of the chemicals remain it can be easily skimmed off. Upon breaking the crust it will be found that the temperature of the molten metal has risen greatly. In this state of great molecular activity caused by the union of the aluminum with oxygen liberated by the potassium bichromate the whole mass becomes thoroughly homogeneous and a true union of the aluminum and other metal or metals results, the union of oxygen with the aluminum producing atomic as well as molecular activity. The action of the borax is to dissolve the oxids as fast as they are formed. In this manner the full benefit of the oxygen is utilized and the presence of objectionable oxids is prevented.

In the compounding of aluminum with copper, if preferred the aluminum may be melted separately from the copper and poured into the molten copper after the addition of the chemicals. If the potassium bichromate or other oxidizing agent and the flux are added before the aluminum, the resulting composite metal will be harder, will more nearly resemble gold and will better stand nitric acid. If the potassium bichromate or other oxidizing agent and the flux are added after the aluminum, the resulting composite metal will be more malleable and

ductile. After the crust is broken up and the molten metal stirred its temperature quickly returns to the normal temperature within the furnace. At this stage of the process phosphorous, magnesium or other kindred deoxidizing agents may or may not be added. We have found in practice that excellent results follow by adding carbon in any convenient form, preferably powdered charcoal. This prevents oxidation of the molten metal from contact with the air. The pot containing the molten metal is now lifted from the furnace, the charcoal or other form of carbon used is skimmed off and a few ounces of ammonium chlorid may be added. The use of ammonium chlorid is not an essential feature of the invention, but we have found in practice that it increases the fluidity of the metal.

20 Before pouring, the quality of the composite metal may be varied by the addition of other metals either singly or collectively. It is obvious that the intense heat evolved by the union of oxygen given off by the pot 25 titanium bichromate with the aluminum may be utilized to great advantage in melting or dissolving the more refractory metals. We have found during our experiments that platinum, gold and silver of the precious 30 metals, and of the basic metals copper, iron, nickel, magnesium, manganese, tungsten, vanadium, chromium, zinc, tin, lead, antimony, cadmium and bismuth may be compounded, either singly or collectively, with aluminum by means of our novel process. 35 For casting purposes we have found that the addition of silicon to the molten metal greatly improves the sharpness of the castings and renders them less liable to corrosion in use.

Having thus described our invention we claim:

1. The process of compounding aluminum with foundation metals which consists in 45 raising the temperature of the foundation metal above the melting point, then adding aluminum, and then adding an oxidizing agent and a flux.

2. The process of compounding aluminum 50 with foundation metals which consists in raising the temperature of the foundation

metal above the melting point, then adding aluminum, then adding an oxidizing agent and a flux and then skimming and stirring.

3. The process of compounding aluminum 55 with foundation metals which consists in raising the temperature of the foundation metal above the melting point, then adding aluminum, then adding a mixture of potassium bichromate and borax and then skimming and stirring.

4. The process of compounding aluminum with foundation metals which consists in raising the temperature of the foundation metal above the melting point, then adding 65 aluminum, then adding an oxidizing agent and a flux, then skimming and stirring and then adding a deoxidizing agent.

5. The process of compounding aluminum with foundation metals which consists in 70 raising the temperature of the foundation metal above the melting point, then adding aluminum, then adding an oxidizing agent and a flux, then stirring and skimming, then adding a deoxidizing agent and then adding 75 ammonium chlorid.

6. The process of compounding aluminum with molten metals which consists in utilizing the union of oxygen with molten aluminum to produce a thorough compounding of 80 the aluminum with the other metal and then adding a deoxidizing agent.

7. The process of compounding aluminum with molten metals which consists in utilizing the union of oxygen with molten aluminum to produce a thorough compounding of 85 the aluminum with the other metal and then adding ammonium chlorid and a deoxidizing agent.

8. The process of compounding aluminum 90 with foundation metals which consists in melting the foundation metal, then adding aluminum thereto and when the aluminum is melted adding an oxidizing agent and a flux.

In testimony whereof we affix our signatures in presence of two witnesses.

JOSEPH GRENVILLE MELLEN.

WILLIAM FRANCIS MELLEN.

Witnesses:

A. M. WOOSTER,  
S. W. ATHERTON.